

Feb. 21, 1939.

R. H. TERRY ET AL

2,147,724

METHOD OF FORMING THIN-WALLED HOLLOW FERROUS CASTINGS

Filed Feb. 7, 1936

2 Sheets-Sheet 1



Fig. 1



Fig. 2



Fig. 3



Fig. 4

Inventors  
Robert H. Terry &  
Alfred L. Boegehold

By Blackmores, Spencer & Finch  
Attorneys

Feb. 21, 1939.

R. H. TERRY ET AL

2,147,724

METHOD OF FORMING THIN-WALLED HOLLOW FERROUS CASTINGS

Filed Feb. 7, 1936

2 Sheets-Sheet 2



Fig. 5



Fig. 6



Fig. 7

Inventors  
Robert H. Terry &  
Alfred L. Boegehold

By Blackmores, Spence & Flick  
Attorneys

## UNITED STATES PATENT OFFICE

2,147,724

METHOD OF FORMING THIN-WALLED  
HOLLOW FERROUS CASTINGS

Robert H. Terry and Alfred L. Boeghold, Detroit,  
Mich., assignors to General Motors Corporation,  
Detroit, Mich., a corporation of Delaware

Application February 7, 1936, Serial No. 62,724

12 Claims. (Cl. 29—148.2)

This invention relates to a process for producing thin-walled hollow shapes. Very often it is desired to construct light weight articles of a complicated shape which are very difficult to make. Such articles may be made by uniting various sheet metal stampings but this process is undesirable due to the excessive cost of dies for the parts. We have found a process by which these thin walled objects may be made by a casting and heat treating process.

In general, the process consists of making a white iron casting similar in composition to the white iron used for making malleable cast iron. This casting is then heated to some temperature between 1600° and 2000° F. in an atmosphere of moist hydrogen for a long enough period to decarburize the surface layer of the casting to a depth equal to the wall thickness desired in the finished shape. This decarburized casting is then drilled in one or two places through the decarburized skin. The holes are then filled with a paste of carbonaceous material and the casting is then again heated to a temperature above the melting point of the undecarburized center of the casting. This melts the inside undecarburized material which bleeds from the hole drilled through the decarburized skin, leaving the low carbon outside skin which forms the hollow object. Hollow thin-walled objects made by this process may be used to advantage as component parts for a copper brazed structure.

The wall material resulting from the process is suitable for copper brazing because it is very low in carbon and behaves in the same way as low carbon steel. It is also free from flake graphite or free carbon in any form and, therefore, does not change in size during the brazing operation in the way that cast iron or malleable iron does.

The specific conditions which have been used in making the hollow articles thus far have been as follows:

A casting has been made containing 2½% carbon, 1.15% silicon and .40% vanadium, .40% manganese, the rest iron, plus usual impurities such as phosphorus and sulphur. In order to obtain a decarburized surface layer .040" deep, the casting was heated for one and one-half hours at 1800° F. in moist hydrogen. Thinner or thicker layers of decarburized irons may be obtained by varying the time and temperature. After having produced the decarburized surface layer, the casting is cooled down and a hole drilled which is plugged with graphite paste in order to prevent decarburization of this hole.

when again heated in hydrogen to melt out the inside. The casting is then heated between 2100° and 2300° F. and held long enough for the core to melt and drain out.

Experiments have been conducted in which the original white iron casting with a drain hole provided in the casting is heated to 1800° F. in the moist hydrogen atmosphere for a period long enough to produce a decarburized layer and then heated on up to above 2100° to melt out the core. 10 This produced a result similar to the above process except that some difficulty in obtaining complete draining was experienced on account of the graphite paste burning out of the drain hole, causing decarburization at the bottom of the 15 hole enough to restrict the draining of the molten core.

Experiments have been conducted with other white iron compositions such as 3½% carbon, ½% silicon, the rest iron, in which the depth of 20 decarburization was not uniform, producing less desirable result than with the composition given above.

Another test with the above given first composition without the vanadium did not drain satisfactorily so that it appears that the presence of the vanadium is instrumental in producing the best results.

Very good results have been obtained from the use of iron carbon alloy castings. 30

On the drawings

Figure 1 shows a section through a conventional furnace with the casting of the invention therein.

Figure 2 is a section through the casting after 35 the outer skin or layer has been decarburized.

Figure 3 is a similar section but showing the opening or cavity made in the carburized casting.

Figure 4 is a view similar to Figures 2 and 3 but 40 showing the graphite plug in the cavity.

Figure 5 is a view similar to Figure 1 but showing the decarburized casting replaced in the furnace and showing the openings with the metal 45 running therefrom.

Figure 6 is a section through a part of the casting after the interior metal has flowed therefrom and the casting cooled.

Figure 7 is a perspective view with parts broken 50 away to show the finished casting.

On the drawing the numeral 2 indicates a furnace of any suitable type having a door 4, heating element 6, and heat resisting floor member 8. A tube 10 is provided at any suitable point to pro- 55

vide for the inlet of hydrogen gas. The numeral 12 indicates the casting of the invention.

The casting 12 is formed to the shape indicated in Figure 1 by the usual casting methods 5 and prior to its being placed in the furnace is composed of solid cast iron. The particular article in question is the inlet and outlet port for a two-cycle engine having a U-type cylinder. The article is heated in the furnace until the outer 10 layer or skin is decarburized.

In Figures 2, 3, and 4, the casting 12 is shown 15 in section and has the openings 14 to enable the inlet and outlet of gas to and from the cylinders. In these figures, the numeral 16 designates the outer decarburized surface or skin of the casting, while the numeral 18 shows the inner metallic or undecarburized portion, the dotted line showing the line of division between the two. As 20 shown in Figure 3, one or more holes or cavities 20 is provided in the casting after the decarburized surface 16 has been formed thereon and this cavity 20 is later filled with the plug indicated at 22. The material of this plug 22 must 25 comprise a substance or material that will prevent the decarburization of the metal, particularly the metal in the hole. Preferably the plug is composed of a non-fusible carbonaceous material such as a graphite paste.

After the graphite plug or plugs 22 have been 30 applied, the casting is replaced in the furnace as shown in Figure 5 and reheated in an atmosphere of hydrogen or other non-oxidizing atmosphere. The graphite plug will prevent further decarburization of the interior metal at the hole. 35 The temperature is increased until it passes somewhat beyond the fusion point of the metal 18 on the interior, but is never allowed to get high enough to melt the exterior decarburized shell 16. When the desired temperature has 40 been reached the carbonaceous plug 22 will be forced out by the pressure of the molten metal 18 and allow the metal 18 of the interior to flow from the openings, the melted metal being indicated by the numeral 24 in Figure 5. When the 45 interior metal is fused it will have a small amount of expansive force due to its change from the solid to the liquid state. This force probably aids in the pushing out of the graphite plug.

50 After the metal 24 has fused and flowed from the opening or cavity 20 the article is removed and allowed to cool and is then in the shape shown in Figure 7. It will be noted that the casting is hollow, leaving a thin-shelled casting 55 through which water may be freely circulated if desired. The interior or hollow portion 26 in Figures 6 and 7 represents the portion previously occupied by the metal 18 in Figures 2, 3, and 4.

When the hollow castings are taken from the 60 furnace it has been found that at times some of them are very brittle and break easily. This is due to the carburizing action of the undecarburized molten metal from the interior of the casting. When the article is heated to cause the interior metal to flow there is sometimes a carburizing action causing the carbon to penetrate the decarburized surface. This causes the brittleness. The article or casting can subsequently be 65 made ductile by again placing it in a furnace and decarburizing in an atmosphere of moist hydrogen.

The hollow article of the invention may be 70 made without removing the article from the furnace in order to make the hole or cavity. This 75 is accomplished by making a cavity in the cast-

ing before it is put into the furnace. This cavity is then filled with some kind of a material, such as graphite, which is not affected by the heat necessary to decarburize the outer surface of the casting. By controlling the temperature and causing the temperature gradually to rise so that the hydrogen atmosphere will decarburize the exterior, and by then bringing the temperature to a sufficiently high degree, the interior metal will fuse and the weight of the fused metal will 10 push out the plug and allow the metal to flow from the casting. After the metal has run out the process may be continued for a short time thoroughly to decarburize the hollow article.

While the invention has been shown applied to 15 one specific article, it is capable of use in connection with other articles where a light casting is desired.

We claim:

1. The method of forming a thin-shelled article or casting consisting of heating an iron carbon alloy casting in an atmosphere of moist hydrogen to cause the decarburization of the surface of the casting, allowing the casting to cool, making a cavity or hole in the casting, filling the hole with a substance capable of preventing the decarburization of the casting at the hole, then in reheating the casting to a temperature above the fusion temperature of the metal inside the casting to cause the molten metal to 30 force the filled substance from the casting to enable the metal to flow and leave a hollow article.

2. The method of forming a thin-shelled casting consisting of heating a casting in an atmosphere of moist hydrogen to a temperature to cause the decarburization of the surface of the casting, allowing the casting to cool sufficiently to enable the placing of a hole or cavity therein, making a cavity or hole in the member, filling the cavity with a material capable of preventing the decarburization of the casting at the hole, then in reheating the casting in a hydrogen atmosphere to a temperature which is lower than the fusion point of the decarburized surface but higher than the fusion point of the interior undecarburized metal thereby to cause the undecarburized metal to fuse and force the filled material from the hole to enable the metal to flow from the casting and leave a hollow article.

3. The method of forming a thin-shelled article consisting of decarburizing the surface of a member, allowing the member to cool, making a cavity or hole in the member, filling the hole with a substance capable of preventing the decarburization of the member at the hole, then in heating the member in a non-oxidizing atmosphere to a temperature lower than the fusion temperature of the decarburized metal but greater than the temperature of fusion of the metal 60 inside the member to cause the weight of the molten interior metal to force the filled substance from the hole to enable the interior metal to flow from the member and leave a hollow article.

4. The method of forming a thin-shelled article consisting of heating a metallic member in an atmosphere of moist hydrogen to a temperature to cause the decarburization of the surface of the member, allowing the member to cool sufficiently to enable the placing of the hole or cavity therein, making a cavity or hole in the member, filling the cavity with a material capable of preventing the decarburization of the member at the hole, then in reheating the mem- 75

ber in a hydrogen atmosphere to a temperature which is lower than the fusion point of the decarburized surface but higher than the fusion point of the interior metal to cause the molten metal to force the filled material from the hole to enable the metal to flow from the casting and leave a hollow article.

5. The method of forming a thin-shelled casting consisting of heating a casting in an atmosphere of moist hydrogen to a temperature to cause the decarburization of the surface of the casting, allowing the casting to cool sufficiently to enable the making of a hole or cavity therein, making a cavity or hole in the member, filling the cavity with a material capable of preventing the decarburization of the casting at the hole, then in reheating the casting in a hydrogen atmosphere to a temperature which is lower than the fusion point of the decarburized surface but higher than the fusion point of the interior undecarburized metal thereby to cause the undecarburized metal to fuse and force the filled material from the hole to enable the metal to flow from the casting and leave a hollow article and then reheating the hollow article in a non-oxidizing atmosphere to decarburize the article.

6. The method of forming a thin-shelled article consisting of decarburizing the surface of a member, allowing the member to cool, making a cavity or hole in the member, filling the hole with a substance capable of preventing the decarburization of the member at the hole, then in heating the member in a non-oxidizing atmosphere to a temperature lower than the fusion temperature of the decarburized metal but greater than the temperature of fusion of the metal inside the member to cause the weight of the molten interior metal to force the filled substance from the cavity to enable the interior metal to flow from the member and leave a hollow article, and then reheating the hollow article in a non-oxidizing atmosphere to decarburize the article.

7. The method of forming a thin-shelled article consisting of heating a metallic member in an atmosphere of moist hydrogen to a temperature to cause the decarburization of the surface of the member, allowing the member to cool sufficiently to enable the making of the hole or cavity therein, making a cavity or hole in the member, filling the hole with a material capable of preventing the decarburization of the member at the hole, then in reheating the member in a hydrogen atmosphere to a temperature which is lower than the fusion point of the decarburized surface but higher than the fusion point of the interior metal to cause the molten metal to force the filled material from the cavity to enable the metal to flow from the casting and leave a hollow article, and then reheating the hollow article in a non-oxidizing atmosphere to decarburize the article.

8. The method of forming a thin-shelled article or casting consisting of forming a cavity or recess in a casting, filling the cavity with a difficultly fusible or non-fusible substance, then in gradually heating the casting in an atmosphere

of moist hydrogen to cause the decarburization of the surface of the casting, then in raising the temperature of the casting to a temperature above the fusion temperature of the metal inside the casting to cause the molten metal to force the filled substance from the casting to enable the metal to flow and leave a hollow article.

9. The method of forming a thin-shelled casting consisting of forming a cavity or recess in the casting, filling the cavity with a difficultly fusible or non-fusible substance, then in gradually heating the casting in an atmosphere of moist hydrogen to a temperature to cause the decarburization of the surface of the casting, then in heating the casting to a temperature which is lower than the fusion point of the decarburized surface but higher than the fusion point of the interior undecarburized metal thereby to cause the undecarburized metal to fuse and force the filled material from the cavity to enable the metal to flow from the casting and leave a hollow article.

10. The method of forming a thin-shelled ferrous article consisting of forming a cavity or recess in a ferrous member, filling the cavity with a difficultly fusible or non-fusible substance, then in decarburizing the surface of the member, then in heating the member in the non-oxidizing atmosphere to a temperature lower than the fusion temperature of the decarburized metal but greater than the temperature of fusion of the metal inside the member to cause the weight of the molten interior metal to force the filled substance from the cavity to enable the interior metal to flow from the member and leave a hollow article.

11. The method of forming a thin-shelled ferrous article consisting of forming a cavity or recess in a ferrous member, filling the cavity with a difficultly fusible or non-fusible substance, then in gradually heating the member in an atmosphere of moist hydrogen to a temperature to cause the decarburization of the surface of the member, then in heating the member in the hydrogen atmosphere to a temperature which is lower than the fusion point of the decarburized surface but higher than the fusion point of the interior metal to cause the molten metal to force the filled material from the cavity to enable the metal to flow from the casting and leave a hollow article.

12. The method of forming a thin-shelled article or casting consisting of heating an iron carbon alloy casting in an atmosphere of moist hydrogen to cause the decarburization of the surface of the casting, allowing the casting to cool, making a cavity or hole in the casting, filling the hole with graphite, then in reheating the casting to a temperature above the fusion temperature of the metal inside the casting to cause the molten metal to force the graphite from the casting to enable the metal to flow and leave a hollow article.

ROBERT H. TERRY.  
ALFRED L. BOEGEHOOLD.